



US008016633B2

(12) **United States Patent**  
**Jiang et al.**

(10) **Patent No.:** **US 8,016,633 B2**  
(45) **Date of Patent:** **Sep. 13, 2011**

(54) **METHOD FOR MAKING FIELD EMISSION DEVICE INCORPORATING A CARBON NANOTUBE YARN**

(75) Inventors: **Kai-Li Jiang**, Beijing (CN); **Yang Wei**, Beijing (CN); **Peng Liu**, Beijing (CN); **Liang Liu**, Beijing (CN); **Shou-Shan Fan**, Beijing (CN)

(73) Assignees: **Beijing FUNATE Innovation Technology Co., Ltd.**, Beijing (CN); **Hon Hai Precision Industry Co., Ltd.**, Tu-Cheng, New Taipei (TW)

(\*) Notice: Subject to any disclaimer, the term of this patent is extended or adjusted under 35 U.S.C. 154(b) by 236 days.

(21) Appl. No.: **12/583,408**

(22) Filed: **Aug. 20, 2009**

(65) **Prior Publication Data**

US 2009/0311940 A1 Dec. 17, 2009

**Related U.S. Application Data**

(62) Division of application No. 11/434,382, filed on May 15, 2006, now Pat. No. 7,586,249.

(30) **Foreign Application Priority Data**

Sep. 30, 2005 (CN) ..... 2005 1 0100089

(51) **Int. Cl.**

**H01J 9/02** (2006.01)

**H01J 9/18** (2006.01)

(52) **U.S. Cl.** ..... **445/51; 445/50; 445/24; 977/842; 977/882**

(58) **Field of Classification Search** ..... 445/24-5, 445/49-51; 977/842, 882; 313/309-311  
See application file for complete search history.

(56) **References Cited**

**U.S. PATENT DOCUMENTS**

|              |      |         |                          |         |
|--------------|------|---------|--------------------------|---------|
| 7,550,907    | B2 * | 6/2009  | Jiang et al. ....        | 313/309 |
| 2001/0024078 | A1 * | 9/2001  | Dimitrijevic et al. .... | 313/311 |
| 2002/0104603 | A1   | 8/2002  | Chang et al.             |         |
| 2002/0175618 | A1   | 11/2002 | Lee et al.               |         |
| 2004/0051432 | A1 * | 3/2004  | Jiang et al. ....        | 313/311 |
| 2004/0053780 | A1   | 3/2004  | Jiang et al.             |         |
| 2006/0066202 | A1 * | 3/2006  | Manohara et al. ....     | 313/311 |
| 2007/0228920 | A1 * | 10/2007 | Jiang et al. ....        | 313/315 |

**FOREIGN PATENT DOCUMENTS**

|    |            |        |
|----|------------|--------|
| JP | 2000251614 | 9/2000 |
| JP | 2001076651 | 3/2001 |

**OTHER PUBLICATIONS**

KaiLi Jiang et al. Spinning continuous carbon nanotube yarns, Nature Publishing Group, Oct. 24, 2002, vol. 419.

\* cited by examiner

*Primary Examiner* — Mariceli Santiago

(74) *Attorney, Agent, or Firm* — Altis Law Group, Inc.

(57) **ABSTRACT**

A method for making a field emission device includes the following steps. A base and at least one carbon nanotube yarn are provided. The at least one carbon nanotube yarn is attached to the base. The at least one carbon nanotube yarn includes a plurality of carbon nanotube segments. The carbon nanotube segments are joined end to end by van der Waals attractive force.

**9 Claims, 4 Drawing Sheets**

20



10



FIG. 1



FIG. 2



FIG. 3



FIG. 4

## 1

**METHOD FOR MAKING FIELD EMISSION  
DEVICE INCORPORATING A CARBON  
NANOTUBE YARN**

**RELATED APPLICATION**

This application is a divisional of application Ser. No. 11/434,382, filed May 15, 2006, now U.S. Pat. No. 7,586,249, issued Sep. 8, 2009.

This is a divisional application of application Ser. No. 11/434,382, filed May 15, 2006 and entitled "FIELD EMISSION DEVICE AND METHOD FOR MAKING THE SAME".

**BACKGROUND**

**1. Technical Field**

The present invention relates to field emission devices, and particularly to a method for making the field emission device using carbon nanotube yarns as an emitter.

**2. Description of the Related Art**

Field emission materials are used in a variety of application such as flat panel displays to emit electrons. Typical field emission materials include, for example, molybdenum (Mo), tantalum (Ta), silicon (Si), and diamond. However, such materials need high emission voltages to emit electrons, and cannot carry high electric current reliably. Carbon nanotubes typically have superior performance including, in particular, good electron emission capability at low emission voltages, generally less than 100 volts. Furthermore, carbon nanotubes can carry high electric current reliably. Due to these properties, carbon nanotubes are considered to be an ideal field emission material for a variety of applications, especially in field emission displays.

Carbon nanotube-based field emission devices typically include a base acting as a cathode plate, and a carbon nanotube array acting as an emitter formed on the base. Methods for forming the carbon nanotube array on the base typically include mechanical means and *in situ* growth. The mechanical means consists of fixing carbon nanotubes onto the base with chemical agglutinant using a robot arm. Such a mechanical means is time consuming and difficult to operate. Furthermore, it is impossible to manipulate the carbon nanotubes with a diameter smaller than about 1 nanometer (nm).

The *in situ* growth process is generally performed as follows. Firstly, a catalyst film is deposited on a base. The base has a driving circuit preformed thereon. Secondly, a carbon nanotube array is grown on the base by a chemical vapor deposition (CVD) process. However, the carbon nanotube array is generally fabricated under a temperature in the range from 500 degrees centigrade to 900 degrees centigrade. As a result, the driving circuit on the base may be damaged.

**BRIEF DESCRIPTION OF THE DRAWINGS**

The above-mentioned and other features and advantages of the field emission device, and the manner of attaining them, will become more apparent and the invention will be better understood by reference to the following description of embodiments thereof taken in conjunction with the accompanying drawings. The components in the drawings are not necessarily drawn to scale, the emphasis instead being placed upon clearly illustrating the principles of the present apparatus and method. Moreover, in the drawings, like reference numerals designate corresponding parts throughout the several views.

## 2

FIG. 1 is a schematic, isometric view of a field emission device employing one carbon nanotube yarn as an emitter according to a first preferred embodiment;

FIG. 2 is a flow chart of one embodiment of a method for fabricating the field emission device of FIG. 1.

FIG. 3 is a schematic, isometric view of a field emission device employing a number of carbon nanotube yarns as emitters according to a second preferred embodiment; and

FIG. 4 is a schematic, isometric view of a field emission device according to a third preferred embodiment.

Corresponding reference characters indicate corresponding parts throughout the several views. The exemplifications set out herein illustrate at least one preferred embodiment of the invention, in one form, and such exemplifications are not to be construed as limiting the scope of the invention in any manner.

**DETAILED DESCRIPTION OF PREFERRED  
EMBODIMENTS**

Reference will now be made to the drawings to describe in detail the preferred embodiments of the present field emission device and a method for making thereof.

In order to improve manipulability, macroscopic carbon nanotube structures are proposed for use as emitters in the present embodiment. Assembling carbon nanotubes into macroscopic structures is of great importance to their applications at the macroscopic level.

That a long macroscopic carbon nanotube yarn can be drawn out from a superaligned carbon nanotube array has been disclosed in US Pub. No. 20040053780, which is incorporated herein by reference. A carbon nanotube yarn includes a plurality of carbon nanotube bundles, also known as carbon nanotube segments, that are joined end to end by van der Waals attractive force, and each of the carbon nanotube bundles includes a plurality of carbon nanotubes substantially parallel to each other. Each carbon nanotube bundle is joined with the carbon nanotubes adjacent to it at either end in a sideward direction instead of longitudinal direction, along an axial direction of the carbon nanotube of each of the carbon nanotube bundles. In general, the combined width of the carbon nanotube yarn can be controlled by a size of the tips of the tool that is used to pull out the carbon nanotube yarn. The smaller the tips, the thinner the combined width of the carbon nanotube yarn. A force required to pull out the carbon nanotube yarn together depends on the combined width of the carbon nanotube yarn. For example, a force of 0.1 micro Newton (mN) is needed to pull out a 200  $\mu\text{m}$  wide wire from a superaligned carbon nanotube array. Generally, the greater the combined width of the carbon nanotube yarn, the greater the force required. A combined length of the carbon nanotube yarn depends on an area of the superaligned carbon nanotube array. Experimental data indicates that it may be possible to draw out a 10 meter (m) long 200  $\mu\text{m}$  wide carbon nanotube yarn from a 100  $\mu\text{m}$  high carbon nanotube array having an area of 1  $\text{cm}^2$ .

Referring to FIG. 1, a field emission device 10 according to a first preferred embodiment of the present invention is shown. The field emission device 10 includes a base 12, and one carbon nanotube yarn 14 attached to the base 12. In the present embodiment, the carbon nanotube yarn 14 extends perpendicularly from a top surface of the base 12 and functions as an emitter.

The base 12 may be made of a metal, such as copper (Cu), nickel (Ni), and molybdenum (Mo). In the present embodiment,

ment, the base **12** is made of Cu. The base **12** may be cylinder, cuboid or other shape. The base **12** is a cylinder in the present embodiment.

The carbon nanotube yarn may be mechanically or metallurgically attached to the base. In one embodiment, the field emission device **10** further includes a conductive paste **16** applied between the carbon nanotube yarn **14** and the base **12**, thereby attaching the carbon nanotube yarn **14** to the base **12**. The conductive paste **16** is an electrically conductive material, such as silver paste.

A length of the carbon nanotube yarn **14** is in the range from about 1 millimeter (mm) to about 100 mm, and a width of that is in the range from about 2 microns ( $\mu\text{m}$ ) to about 200  $\mu\text{m}$ . In one embodiment, the carbon nanotube yarn **14** has a length of about 60 mm and a width of about 100  $\mu\text{m}$ .

Referring to FIG. 2, a method for making the field emission device **10** is provided as follows, and includes the steps in no particular order of:

- (1) providing a base **12**;
- (2) providing a super-aligned carbon nanotube array with 100  $\mu\text{m}$  high, 1  $\text{cm}^2$  area, pulling out a carbon nanotube yarn **14** from the super-aligned carbon nanotube array;
- (3) attaching the carbon nanotube yarn **14** to a top surface of the base **12** using silver paste **16**; and
- (4) sintering the silver paste **16** at a temperature of between 400 degrees centigrade and 550 degrees centigrade for about 30 minutes to obtain the field emission device **10** with carbon nanotube yarn **14** extended perpendicularly from the top surface of the base **12**.

It is understood that, in step (2), if the carbon nanotube yarn **14** is long enough, the carbon nanotube yarn **14** can be cut into a plurality of sections/segments, one of which is then selected to serve as the field emitter.

The silver paste **16** should be sintered in air, nitrogen, hydrogen, a mixture gas thereof, or a gas containing less than 30% of oxygen. Alternatively, the carbon nanotube yarn could be mechanically or metallurgically attached to the base. The carbon nanotube yarn may be attached on the base **12** and extend coaxially with the base **12**.

The field emission device **10** can emit an electric current with 50 mA or above when a voltage of about 500V to 1000V is applied between the field emission device **10** and an anode electrode disposed 10 mm distant from the field emission device **10**.

It is understood that we can use a plurality of carbon nanotube yarns as emitters under the same condition. Referring to FIG. 3, a field emission device **20** of another embodiment is shown. The field emission device **20** includes a columniform base **22** made of Cu, and a plurality of carbon nanotube yarns **24** attached to the base **22** and extending perpendicularly from a top surface of it. A conductive silver paste **26** is applied between the carbon nanotube yarns **24** and the base **22**, thereby attaching the carbon nanotube yarns **24** to the base **22**.

Referring to FIG. 4, a field emission device **30** having a plurality of carbon nanotube yarns as emitters according to other one embodiment is shown. The field emission device **30** includes a columniform base **32** made of Cu, a plurality of carbon nanotube yarns **34** with 100 mm length and 200  $\mu\text{m}$  width attached to the side surface of the base **32**, and a layer of conductive silver paste **36** applied between the carbon nanotube yarns **34** and the base **32** for attaching the carbon nanotube yarns **34** to the base **32**. In one embodiment, the carbon nanotube yarns **34** extend from a side surface of the base **32**. This configuration makes good use of the side sur-

face area of the base **32** so as to enlarge a contact area between the carbon nanotube yarns **34** and the base **32**.

The field emission device and method according to the present invention has the following advantages. Firstly, the carbon nanotube yarns as field emitters of the field emission device can emit high electric current reliably. Secondly, in the present method, the at least one carbon nanotube yarn is attached to a base using a conductive paste. The conductive paste is then sintered for fixing the at least one nanotube to the base. The temperature for sintering the conductive paste is generally in a range of 400 degrees centigrade to 550 degrees centigrade and is far lower than the operation temperature of 500 degrees centigrade to 900 degrees centigrade in the conventional in situ growth method. This avoids damage of the driving circuit on the base.

While the present invention has been described as having preferred or exemplary embodiments, the embodiments can be further modified within the spirit and scope of this disclosure. This application is therefore intended to cover any variations, uses, or adaptations of the embodiments using the general principles of the disclosure as claimed. Furthermore, this application is intended to cover such departures from the present disclosure as come within known or customary practice in the art to which the invention pertains and which fall within the limits of the appended claims or equivalents thereof.

What is claimed is:

1. A method for making a field emission device, the method comprising:

- (a) providing a base and at least one carbon nanotube yarn, the at least one carbon nanotube yarn comprising a plurality of carbon nanotube segments, the carbon nanotube segments are joined end to end by van der Waals attractive force; and
- (b) attaching the at least one carbon nanotube yarn to the base.

2. The method as described in claim 1, wherein in step (b), the at least one carbon nanotube yarn is mechanically or metallurgically attached to the base.

3. The method as described in claim 1, wherein, in step (b), the at least one carbon nanotube yarn is attached to the base using conductive paste.

4. The method as described in claim 3, wherein the conductive paste comprises a silver paste.

5. The method as described in claim 3, further comprising a step of sintering the conductive paste thereby securing the at least one carbon nanotube yarn to the base.

6. The method as described in claim 5, wherein the conductive paste is sintered at a temperature in the range from 400 degrees centigrade to 550 degrees centigrade, for over 30 minutes.

7. The method as described in claim 1, wherein the at least one carbon nanotube yarn is obtained by a method comprising the steps of:

- (a) providing a super-aligned carbon nanotube array; and
- (b) drawing out a carbon nanotube segments from said super-aligned carbon nanotube array such that a carbon nanotube yarn is formed.

8. The method as described in claim 1, wherein a length of the carbon nanotube yarn is in the range from about 1 mm to about 100 mm.

9. The method as described in claim 1, wherein a width of the carbon nanotube yarn is in the range from about 2  $\mu\text{m}$  to about 200  $\mu\text{m}$ .